# EUROPEAN PATENT APPLICATION

(11) **EP 4 183 894 A1**
(43) Date of publication of application: **24.05.2023**
(21) Application number: 22208081.4
(22) Date of filing: 17.11.2022
(51) Int. Cl.: C23C 18/00, H01L 21/00, H01R 13/03

(54) **METHOD FOR SURFACE TREATMENT OF AN ELECTRICAL CONTACT ELEMENT AND CONTACT ELEMENT**

(30) Priority: 18.11.2021 DE 102021130188
(71) Applicant: TE Connectivity Germany GmbH, 64625 Bensheim (DE)
(72) Inventor: Greiner, Felix, 64625 Bensheim (DE); Thoss, Stefan, 64625 Bensheim (DE); Leidner, Michael, 67346 Speyer (DE); Ostendorf, Frank, 64625 Bensheim (DE); Schmidt, Helge, 67346 Speyer (DE); Sanchez, Esteban, 67346 Speyer (DE); Job, Stefan, 67346 Speyer (DE)
(74) Representative: Grünecker Patent- und Rechtsanwälte PartG mbB

(57) **Abstract**

The present invention relates to a method for surface treatment of an electrically conductive contact element (100, 200) for an electrical connector (300, 400) by means of plasma, wherein a lubricant (106, 206) is applied to at least a partial region of the contact surface (102, 202). Furthermore, the invention relates to an electrically conductive contact element (100, 200) whose surface is treated by means of such a method. The method for surface treatment of an electrically conductive contact element (100, 200) for an electrical connector (300, 400) relates to an electrically conductive contact element (100, 200) which has a metallic contact surface (102, 202) and to which a lubricant (106, 206) is applied at least in a partial region of the contact surface (102, 202) of the electrically conductive contact element (100, 200). Furthermore, the contact surface (102, 202) of the electrically conductive contact element (100, 200) is changed by means of plasma treatment, whereby a coating (120) of a solid lubricant is produced at least in sections on at least a partial region of the contact surface (102, 202) of the electrically conductive contact element (100, 200).

## Description

The present invention relates to a method for surface treatment of an electrically conductive contact element for an electrical connector. Furthermore, the invention relates to an electrically conductive contact element whose surface is treated by means of such a method.

Electrical connectors and their contact elements are known in numerous designs. Electrical connectors are intended to be mated with a suitable mating connector to establish an electrical connection. Electrical connectors are generally used either for signal transmission or for power transmission. For this purpose, electrical connectors generally have electrically conductive contact elements that come into contact with a contact element of the mating connector when the connector is mated. Frequently, the contact elements of one connector element are designed as contact pins and those of the mating connector as contact springs. When the connector and mating connector are mated, the contact springs exert elastic spring forces on the contact pins to ensure a reliable electrically conductive connection.

Electrical connectors are used in motor vehicles, for example, to transmit power and network electrical and electronic systems. In motor vehicles, connectors are exposed to strong temperature fluctuations, vibrations, moisture and corrosive media. An increase in operating temperatures results in increased wear, particularly in the case of the widely used tin-plated copper-based contact elements.

In particular, base metal contact surfaces, e.g. with tin, nickel or their alloys, have a tendency to fretting corrosion ("fretting" or "scuffing") in the event of small relative movements. Furthermore, in the case of high-pole connectors, the mating forces are often outside the required forces, especially during initial mating, and in the case of noble contact surfaces, e.g. noble metal-based, the tendency to cold welding represents a known problem.

In addition to high wear resistance, low mating and drawing forces are therefore required to facilitate the assembly and maintenance of connectors. To increase occupational safety, the specified mating force must not exceed certain limits, especially during initial mating.

In addition, partial abrasion takes place on the contact surface of a contact element during mating of a connector with a mating connector. This wear caused by abrasion limits the mating frequency of connectors and thus reduces their operating times.

The German patent specification DE 10 2016 214 693 B4 describes an electrical contact element of a connector in which caverns filled with an auxiliary material are arranged under the contact surface. The contact surface was previously textured by laser irradiation. After the connector has been mated for the first time into a mating connector, the caverns break open causing the auxiliary material to escape and to cover the contact surface with a lubricating film. This lubricating film results in reduced mating force when the connector is mated again. The treatment of a surface with an interference pattern from laser radiation, in which exemplarily a dimpled structure is created, is referred to below as a textured surface.

However, assembly boundary conditions also define standards for the mating force when the connector is first mated with a mating connector. This initial mating force is of particular importance when assembling connectors with a high number of contacts. There is an additional requirement for the contact surface of the connector to be heat-resistant, as the connectors can also be further processed in warm regions. Applying a lubricating film to the contact surface of the connector is therefore not a suitable solution, as the lubricating film would evaporate at warm temperatures.

Therefore, there is a need for a cost-effective and reliable process that treats the contact surface of an electrical connector in such a way that the initial mating force can be reduced when mating with a mating connector, and the surface treatment does not lose its effect even under adverse environmental conditions.

This task is solved by the subject-matter of the independent claims. Advantageous embodiments of the present invention are the subject matter of the dependent claims.

In this context, the present invention is based on the idea that improved surface properties of the contact surface of the electrical connector are achieved by treatment with plasma. For this purpose, a lubricant is first applied to the contact surface so that a coating of a solid lubricant is produced on the contact surface by the plasma treatment.

In particular, the present invention comprises a method for surface treatment of an electrically conductive contact element for an electrical connector, wherein the electrically conductive contact element has a metallic contact surface. In addition, a lubricant is applied to at least a partial region of the contact surface of the electrically conductive contact element. Furthermore, the contact surface of the electrically conductive contact element is changed by means of plasma treatment, whereby a coating of a solid lubricant is produced at least in sections on at least a partial region of the contact surface of the electrically conductive contact element.

The coating of a solid lubricant can be, for example, carbon, carbonaceous, or sulfide-based. A carbon layer is understood to be a thin layer consisting predominantly of the chemical element carbon. This includes, for example, graphite layers or diamond-like carbon layers. The applied lubricant layer, which serves as the initial lubricant layer, can be, for example, an oil, grease, paste, or another solid lubricant such as graphite, carbon nanotubes, MoS₂ or mixtures thereof, which is modified by the plasma treatment.

The surface treatment can reduce the roughness of the contact surface of the electrical connector and achieve a higher homogeneity. In addition, the hardness of the contact surface can be increased, e.g. by selectively creating intermetallic phases IMPs or a nanocrystalline microstructure. Each of these improved properties, independent of the others, reduces the initial mating force when mating the connector with a mating connector. In addition, the variations in the coefficient of friction over the entire contact surface can be reduced.

According to an advantageous further development of the present invention, the contact surface of the electrically conductive contact element has a surface texture consisting of elevations and recesses, so that the lubricant applied to the contact surface adheres particularly well.

The plasma is excited in a pressure range from 1 mbar to 8 bar, which means that, advantageously, no vacuum chamber is required for the plasma treatment, which can instead be carried out using atmospheric pressure plasma. This has the advantage that liquid chemicals can be dispensed with entirely. For this purpose, non-hazardous gases such as nitrogen or compressed air can be used for plasma generation. Alternatively, the plasma can be excited under low vacuum or slight overpressure.

In the following, a plasma is understood to be partially or completely ionized gas. The cold or hot plasma is generated and spread by a plasma nozzle directed at the material. Inside the nozzle, the plasma is generated by high voltage between a stator and a rotor. Through an arc-like high-voltage discharge, the ionized gas is directed onto the surface to be treated. For example, hydrogen, argon, nitrogen or compressed air can be used as the gas to be ionized.

Advantageously, the power of the plasma is in the range of 50 W to 5 kW to produce the previously mentioned coating of a solid lubricant from the applied lubricant layer.

According to an advantageous further development of the present invention, caverns filled with an auxiliary material are enclosed under the contact surface of the electrically conductive contact element. These filled caverns break open in the course of the first mating of the connector with a mating connector, allowing the auxiliary material to escape and develop its effect. This allows the mating force to be reduced in the first mating process and even more so for all subsequent mating processes.

An auxiliary material, also called an additive, is a substance that is added in rather small quantities to achieve or improve certain properties.

A cavern is understood to be an artificially created cavity below the surface. The arrangement of the caverns below the contact surface means that the caverns do not have an outlet at the contact surface or, at most, an outlet of such narrow dimensions that auxiliary material filled into the caverns cannot be reached without creating a breakthrough from the contact surface into the cavern.

According to another advantageous embodiment of the present invention, the auxiliary material is selected from the group consisting of antioxidants, corrosion inhibitors, lubricants, another solid lubricant, and acids. This group of substances facilitates, after leakage to the contact surface of a connector, the mating of this connector with a mating connector.

According to an advantageous further development of the present invention, the plasma treatment of the electrically conductive contact element is part of a continuous process. This has the advantage that the edges of the contact surface are also treated uniformly. As a result, a uniformly thin layer of a solid lubricant can advantageously be obtained, as a result of which the contact surface has a high degree of homogeneity.

According to an advantageous further development of the present invention, the plasma treatment comprises irradiation with a plasma flame, wherein the dwell time of the electrically conductive contact element in the plasma flame is between 5 ms and 500 ms. The positive effects mentioned above already occur after this short dwell time, whereby high numbers of pieces can be treated in a short time.

According to an advantageous further development of the present invention, the plasma flame exits from a plasma nozzle, with the distance of the contact surface to the plasma nozzle being 5 mm to 100 mm. This targeted plasma treatment allows an easy integration into an existing manufacturing facility and compliance with safety regulations without the need for additional shielding precautions.

According to an advantageous further development of the present invention, the coating of a solid lubricant produced by the plasma treatment has a thickness of 1 nm to 300 nm. This thin coating allows the plasma treatment to be used for a wide variety of connector types, which can be mated with a matching mating connector without having to adjust the dimensions.

According to an advantageous further development of the present invention, the thickness of the lubricant applied to the contact surface of the electrically conductive contact element is between 0.1 µm and 5 µm. The thinly applied layer adheres particularly well to the rough metallic contact surface.

The present invention further relates to an associated electrically conductive contact element for an electrical connector, which has a metallic contact surface. In addition, the contact surface has, at least in sections, a coating of a solid lubricant produced from a lubricant layer by treatment with plasma. This electrically conductive contact element has the advantage of having a lower first mating force from the start than conventional contact elements. In addition, the standard deviation of the coefficient of friction is reduced, which is particularly important for connectors with a high number of contacts.

It is also advantageous if caverns filled with an auxiliary material are enclosed under the contact surface of the electrically conductive contact element. These break open when the contact element first makes contact with a mating contact, the auxiliary material escapes and the mating force can be reduced during the first mating process and even more so for all subsequent mating processes. Due to the fact that the filled caverns are located under the contact surface, negative effects such as gumming can be avoided. In addition, undesirable losses of the auxiliary material due to the solid embedding are excluded.

According to another advantageous embodiment of an electrically conductive contact element, the auxiliary material is selected from the group of antioxidants, corrosion inhibitors, lubricants, another solid lubricant and acids. These substances reduce wear caused by abrasion, which can increase the mating frequency of the connectors.

According to a further advantageous embodiment of an electrically conductive contact element, the metallic contact surface comprises tin, and/or nickel, and/or silver, and/or copper and/or alloys of tin, nickel, silver, copper. These materials are rust and heat resistant whereby a longevity of the connector can be guaranteed.

According to an advantageous further development of the present invention, a square roughness of the surface in the mating direction is less than 0.3 µm. This value is below the measured values for surfaces, which have not been modified by means of plasma treatment according to the invention. Thus, advantageously, a lower roughness could be achieved, resulting in a more uniform surface and thus an improved mating of the connector with the mating connector.

Surface roughness is the degree of unevenness of a solid surface below its shape or waviness, but above the irregularity of crystal lattice structures. Roughness can affect material properties such as friction. One of the roughness characteristics is the square roughness. This can be detected by optical measurement methods. The evaluation of the measurements was based on the DIN EN ISO 4287 and DIN EN ISO 11562 series of standards. For mating a connector with a mating connector, the roughness in the mating direction is of particular importance. Therefore, in the present case, the measurement is aligned to the mating direction. In one embodiment, this alignment can be made along the surface texture. If the surface texture has elevations and recesses, as in the above-mentioned embodiment, the alignment of the measurement takes place along the elevations and recesses.

For a better understanding of the present invention, it will be explained in more detail with reference to the examples of embodiments shown in the following figures. In this context, identical parts are provided with identical reference signs and identical component designations. Furthermore, some features or combinations of features from the different embodiments shown and described may also represent independent, inventive solutions or solutions according to the invention. Showing:
- **Fig. 1**: a schematic sectional view of a contact surface in a first embodiment in a process step according to a method according to the invention, including an enlarged section of the contact surface;
- **Fig. 2**: a schematic sectional view of a contact surface in a further embodiment in a process step according to a method according to the invention;
- **Fig. 3**: a schematic representation of the surface treatment of a first embodiment of the contact surface by means of plasma in a further process step;
- **Fig. 4**: a schematic sectional view of the contact surface of a first embodiment of the contact surface after plasma treatment in a further process step.

Figure 1 shows, by means of a sectional view of a first embodiment of a contact surface of an electrically conductive contact element, a first process step according to a method according to the invention.

The method is for surface treating an electrically conductive contact element 100. The contact element 100 for an electrical connector 300 is electrically conductive and comprises a base material 104. The base material 104 may comprise, for example, tin, nickel, silver, copper or alloys of tin, nickel, silver, copper and/or other elements. One side of the contact element 100 forms a metallic contact surface 102. The contact surface 102 comes into contact with the contact surface of the mating connector (not shown in the figures) when the connector 300 is mated to a mating connector.

The contact surface 102 is coated on at least a partial region thereof with a lubricant 106. For example, the lubricant 106 may comprise oil, grease, a paste, an acid, or another solid lubricant such as graphite, carbon nanotubes, MoS₂, or mixtures thereof. The thickness of the applied lubricant may have values between 0.1 µm and 5 µm.

In an advantageous embodiment, the contact surface 102 of the contact element 100 may have a surface texture 112 of elevations 124 and recesses 122. These elevations 124 and recesses 122 may be formed periodically alternating at least in sections. In this regard, the recesses 122 form trenches and the elevations 124 form walls between them. The elevations may be in the order of 0.1 µm to 2 µm, by way of example. However, it is by no means necessary for the method according to the invention that the surface texture 112 comprises elevations 124 and recesses 122. It is understood that the contact surface 102 may have any surface texture 112, such as smooth or with other roughness.

Figure 2 shows another embodiment of a contact surface 102 of an electrically conductive contact element 200 in a first process step according to a method according to the invention.

The contact element 200 for an electrical connector 400 is electrically conductive and comprises a base material 204. The base material 204 may comprise, for example, tin, nickel, silver, copper or alloys of tin, nickel, silver, copper and/or other elements. One side of the contact element 200 forms a metallic contact surface 202, and the contact surface 202 comes into contact with the contact surface of the mating connector when the connector 400 is mated with a mating connector.

In the embodiment shown, caverns 208 are enclosed under the contact surface 202 and are filled with an auxiliary material 210. In the embodiment shown, the caverns 208 are spaced apart from each other at regular intervals under the contact surface 202. In this embodiment, the surface texture 212 has exemplary elevations 224 and recesses 222. These elevations 224 and recesses 222 may be formed periodically alternating, at least in sections. In this regard, the recesses 222 form trenches and the elevations 224 form walls between them. The elevations can be in the order of 0.1 µm to 2 µm, by way of example.

It is understood that the caverns 208 may also be irregularly spaced from one another and at varying depths under the contact surface 202. Furthermore, it is also possible for the caverns 208 to be enclosed under the contact surface 202 if the contact surface 202 does not have elevations 224 and recesses 222. For the method according to the invention, it is not necessary that the surface texture 212 comprises elevations 224 and recesses 222. It is understood that the contact surface 202 may have any surface texture 212, such as smooth or with other roughness.

The auxiliary material 210 enclosed in the caverns 208 may comprise, for example, oil, grease, a paste, or another solid lubricant such as graphite, carbon nanotubes, MoS₂ , or mixtures thereof. The contact surface 202 is coated with a lubricant 206 on at least a partial region thereof. For example, the lubricant 206 may comprise oil, grease, a paste, an acid, or another solid lubricant such as graphite, carbon nanotubes, MoS₂ , or mixtures thereof. The thickness of the applied lubricant may have values between 0.1 µm and 5 µm.

Figure 3 shows the contact element 100 according to a first embodiment in a further process step of the method according to the invention.

The figure shows a schematic representation of the surface treatment of the contact element 100 using plasma. In one possible embodiment, a plasma generator 118, for controlling and monitoring the plasma system, is shown schematically with a plasma nozzle 114 directed at the material to be treated. The directed plasma nozzle 114 is used to generate and propagate the plasma. Various nozzle systems, such as single nozzles or rotating nozzles, can be used as plasma sources. From the plasma nozzle 114, a plasma flame 116 is used to treat the contact surface 102. The distance d of the plasma nozzle 114 to the contact surface 102 is in the range of 5 mm to 100 mm.

In this process, it is possible to generate the plasma flame 116 in a pressure range of 1 mbar to 8 bar, thus, for example, treatment of surfaces can also be carried out at atmospheric pressure. The power of the plasma flame 116 is in a range of 50 W to 5 kW. In this case, the treatment of the contact surface 102 is part of a continuous process in which the contact element 100 passes through the plasma flame 116 at a speed of 100 mm/s or 200 mm/s, for example. The dwell time of the contact surface 102 under the plasma flame 116 is then between 5 ms and 500 ms.

It is clear, however, that the values given are only given by way of example and are intended to aid understanding, but in no way limit the invention to these values. Both the passage speed, the distance, and the dwell time can be adjusted as desired and can be adapted to different values of the power of the plasma flame.

Figure 4 shows an exemplary first embodiment of a contact surface 102 of an electrically conductive contact element 100 after surface treatment with plasma. The plasma treatment has produced a coating 120 of a solid lubricant, preferably carbon, on at least a partial region of the contact surface 102. This coating 120 of a solid lubricant may have a thickness of 1 nm to 300 nm and may be transparent. At least part of the applied lubricant from the previous process step thus has been at least partially converted into a coating of a solid lubricant preferably consisting of carbon.

In a second embodiment (not shown), it is quite possible to likewise create a coating 120 of a solid lubricant on the contact surface 202 if, as in a previously mentioned second embodiment of the previous process step, caverns filled with an auxiliary material are enclosed under the contact surface 102. The caverns remain unchanged by the plasma treatment.

Advantageously, in addition to the preferably carbon or carbon-containing coating, the surface properties of the contact element can be improved by the plasma treatment. Accordingly, the treatment reduces unevenness in the contact surface, thus achieving a lower square roughness.

Experimental investigations have shown that the square roughness of a surface after treatment with plasma is less than 0.3 µm. This value is 0.1 µm lower than the value of the square roughness for a surface not treated by means of the process according to the invention.

Advantageously, a higher hardness of the coated surface can additionally be achieved. The hardness of the connector surface can be determined by means of nanoidentification. An indenter with a known geometry is pressed into the surface to be tested with a defined force curve. When the specified maximum force is reached, the indenter is released again in a controlled manner. The indentation depth is recorded both during loading and unloading. Various parameters can be calculated from the applied force, the shape of the indenter and the indentation depth. For a measurement of the surface hardness, at least two measuring points are approached at a predefined distance. The mean value of all measuring points on a surface can be used as a comparable measure of surface hardness. The measurement is first performed on an untreated surface and then a second time after plasma treatment. In an exemplary measurement with 51 measuring points at a distance of 100 µm, an exemplary average hardness value of 450 N/mm² can be determined for the untreated surface. However, for a textured and plasma-treated surface, an exemplary mean value of 750 N/mm² can be determined.

Thus, surfaces exhibit a higher hardness after plasma treatment. When comparing the mean values, an increase in hardness of 40% to 80% can be observed in particular for contact surfaces textured before plasma treatment compared to untreated surfaces.

Finally, a spatially resolved characterization of the plasma-treated surface in terms of roughness, hardness and chemical composition can advantageously reveal a significantly more uniform image than contacts that have been stamped or electroplated, for example.

These advantageous properties occur independently of each other and lead independently of each other to a smaller variation of the coefficient of friction. Within a surface, a narrower distribution of the standard deviation of the coefficient of friction can thus be demonstrated by means of the method according to the invention.

It should be noted that it is quite possible to achieve the same advantageous properties using a different plasma generation method. For example, the plasma flame can be generated in a low-pressure plasma chamber under vacuum.

**List of reference signs:**

| **Reference number** | **Description** |
|---|---|
| 100, 200 | Contact element |
| 102, 202 | Contact surface |
| 104, 204 | Basic material |
| 106, 206 | Lubricant |
| 208 | Cavern |
| 210 | Auxiliary material |
| 112, 212 | Surface texture |
| 114 | Plasma nozzle |
| 116 | Plasma flame |
| 118 | Plasma generator |
| 120 | Coating from a solid lubricant |
| 122, 222 | Recess |
| 124, 224 | Elevation |
| d | Distance of the plasma nozzle to the contact surface |
| 300, 400 | Connector |

## Claims

1. A method for surface treating an electrically conductive contact element (100, 200) for an electrical connector (300, 400),
wherein the electrically conductive contact element (100, 200) comprises a metallic contact surface (102, 202), and
wherein a lubricant (106, 206) is applied to at least a partial region of the contact surface (102, 202) of the electrically conductive contact element (100, 200), and
wherein the contact surface (102, 202) of the electrically conductive contact element (100, 200) is changed by means of plasma treatment, whereby a coating (120) of a solid lubricant is produced at least in sections on at least a partial region of the contact surface (102, 202) of the electrically conductive contact element (100, 200).

2. The method according to claim 1,
wherein the contact surface (102, 202) of the electrically conductive contact element (100, 200) has a surface texture of elevations (124, 224) and recesses (122, 222).

3. The method according to any one of the preceding claims,
wherein the plasma is excited in a pressure range from 1 mbar to 8 bar.

4. The method according to any one of the preceding claims,
wherein the power of the plasma is in the range of 50 W to 5 kW.

5. The method according to any one of the preceding claims,
wherein caverns (208) filled with an auxiliary material (210) are enclosed under the contact surface (102, 202) of the electrically conductive contact element (100, 200).

6. The method according to any one of the preceding claims,
wherein the auxiliary material (210) is selected from the group consisting of antioxidants, corrosion inhibitors, lubricants, another solid lubricant, and acids.

7. The method according to any one of the preceding claims,
wherein the plasma treatment of the electrically conductive contact element (100, 200) is part of a continuous process.

8. The method according to any one of the preceding claims,
wherein the plasma treatment comprises irradiation with a plasma flame (116), and
wherein the dwell time of the electrically conductive contact element (100, 200) in the plasma flame (116) is between 5 ms and 500 ms.

9. The method of claim 8,
wherein the plasma flame (116) exits from a plasma nozzle (114), and
wherein the distance of the contact surface to the plasma nozzle (114) is 5 mm to 100 mm.

10. The method according to any one of the preceding claims,
wherein the coating (120) of a solid lubricant produced by the plasma treatment has a thickness of 1 nm to 300 nm.

11. The method according to any one of the preceding claims,
wherein the thickness of the lubricant (106, 206) applied to the contact surface (102, 202) of the electrically conductive contact element (100, 200) is between 0.1 µm and 5 µm.

12. Electrically conductive contact element (100, 200) for an electrical connector (300, 400),
which has a metallic contact surface (102, 202),
wherein the contact surface (102, 202) has, at least in sections, a coating (120) of a solid lubricant produced by treatment with plasma from a lubricant layer (106, 206).

13. An electrically conductive contact element (100, 200) according to claim 12,
wherein caverns (208) filled with an auxiliary material (210) are enclosed below the contact surface (102, 202).

14. An electrically conductive contact element (100, 200) according to any one of claims 12 or 13,
wherein said auxiliary material (210) is selected from the group consisting of antioxidants, corrosion inhibitors, lubricants, another solid lubricant, and acids.

15. An electrically conductive contact element (100, 200) according to any one of claims 12 to 14,
wherein the metallic contact surface (102, 202) comprises tin, and/or nickel, and/or silver, and/or copper, and/or alloys of tin, nickel, silver, copper.

16. An electrically conductive contact element (100, 200) according to any one of claims 12 to 15,
wherein a square roughness of the surface in the mating direction is less than 0.3 µm.
